

M. B. BECKER.  
PREPARED ROOFING.  
APPLICATION FILED MAY 3, 1913.

1,157,665.

Patented Oct. 26, 1915.

*Fig. 1.*



*Fig. 2.*



*Fig. 3.*



WITNESSES:

R. G. Fanning

M. M. Boyle

Mathias B. Becker  
By *John Scheible, Atty.*

# UNITED STATES PATENT OFFICE.

MATHIAS B. BECKER, OF CHICAGO, ILLINOIS.

## PREPARED ROOFING.

1,157,665.

Specification of Letters Patent.

Patented Oct. 26, 1915.

Application filed May 3, 1913. Serial No. 765,309.

*To all whom it may concern:*

Be it known that I, MATHIAS B. BECKER, citizen of the United States, residing at Chicago, in the county of Cook and State 5 of Illinois, have invented certain new and useful Improvements in Prepared Roofing; and I do hereby declare the following to be a full, clear, and exact description of the invention, such as will enable others skilled 10 in the art to which it appertains to make and use the same.

This invention has for its object to provide prepared roofing of the character that is made in the factory and marketed in rolls 15 ready to lay, which has its surface coated with grit of contrasting colors relatively arranged and disposed to form a predetermined pattern or design on the weather face of the material whereby it will be given an 20 ornamental appearance similar, for example, to that of a tile or shingle roof.

Roofing embodying my invention is illustrated in the accompanying drawings in which:

25 Figure —1— is a view in elevation of the weather face of roofing having contrasting grit coatings applied thereto whereby the same is given an ornamental appearance. Fig. —2— is a fragmentary cross section of 30 the same on the line 2—2 of Fig. —1—. Fig. —3— is a fragmentary detail sectional view on an enlarged scale similar to Fig. —2—.

The commercial prepared roofing to which 35 my invention relates is made in very large quantities and is very cheap, consisting of a base or web of wool-felt, paper or other porous or fibrous material which is passed through a vat of boiling asphaltic material 40 with which it becomes coated and impregnated. As it leaves the tank the roofing passes over a roll or rolls and upon the upper face thereof mineral grit is dropped or projected. This grit consists of gravel, 45 crushed stone, slate, brick or any similar suitable material, and, being applied while the asphaltic surface is very soft, it becomes partially embedded therein and gives to the surface of the roofing the general color 50 effect of the grit particles. This color effect is, however, uniform over the entire surface and is rather monotonous.

The object of my present invention is to provide a roofing having on its surface a plurality of grit coatings of contrasting

colors relatively arranged and disposed so that the contrasting colors will display a predetermined design or pattern on the roofing.

To this end I apply to the roofing after 60 the primary coating of grit has been applied to its surface and upon and over said grit coating, a second coating preferably of asphaltic material in pattern form so as to produce the desired design or pattern thereon. This second coating is applied in liquid 65 form in such quantity as to penetrate through the grit coating and upon the asphaltic base or coating holding said grit. Said second coating is of such a nature that 70 it will amalgamate with and become inseparable from the lower coating. This is accomplished, preferably, in the manner and by the means fully described in Letters Patent No. 1,024,549 and No. 1,024,550 is- 75 sued to me on April 30, 1912.

While the pattern coating is still soft and fluent I project thereon in any suitable manner, grit of any suitable nature and of a 80 color contrasting with that of the primary grit coating and which becomes partially embedded in the pattern coating and is held thereby, any unapplied surplus of said last-named grit being shaken off and recovered 85 in any suitable manner.

In the accompanying drawings which 90 illustrate roofing embodying the invention as fully as the nature of the material admits, A indicates the porous or fibrous web and B and C the asphaltic coatings covering and impregnating said web. To the coating B the grit particles D are applied, the latter being of a uniform color and becoming 95 partially embedded in said coating B and held thereby. The pattern coating E applied over and penetrating through the coating of grit particles D is shown to be homogeneous with the coating B and upon the same the grit particles F are applied which 100 are of any suitable color contrasting sharply with the color of the particles D. The said particles F afford a protective coating for the pattern material and serve also to prevent the latter from adhering to the coating C when the roofing is rolled up ready for 105 shipment.

I claim as my invention:

1. A ready-to-lay roofing comprising a base of water-proof material, and an ornamental protecting face formed of exposed 110

- differently colored grits relatively disposed at different elevations to present a desired design and intimately united with the base to form a permanent part thereof.
5. 2. A ready-to-lay roofing comprising a base of waterproofing material having a surface of relatively raised and depressed portions bearing a protecting face formed of exposed grits, the grit on the raised portions differing in appearance from the grit in the depressed portions to present a predetermined symmetrical design, ultimately, united with the base to form a permanent part thereof.
10. 3. Prepared roofing comprising a web coated and impregnated with a weather resisting material, the coating on one face of the web being varied in thickness in various parts or fields, a coating of granular grit of a uniform color partially embedded in the fields of least thickness and extending through and completely embedded in the parts or fields of greater thickness, and a coating of granular grit of a color contrasting with the color of the first-named grit coating partially embedded in the parts or fields of greater thickness.
15. 4. A roofing material comprising a base having on its face a layer of protecting grit, a superposed layer of similar protecting ma-
- terial, and a suitable binder interposed therebetween.
5. A roofing material comprising a base having relatively thick and thin portions, the thicker portions having protecting grit 35 on its face and similar grit interposed between the upper and lower surfaces of the base and completely embedded therein.
6. A roofing material comprising a base having relatively thick and thin portions, 40 the thicker portions having protecting grit on its face and sides, and similar grit interposed between the upper and lower surfaces of the base and completely embedded therein.
7. A roofing material comprising a base having on its face relatively depressed portions, a layer of grit substantially exposed to protect the same, and relatively elevated portions similarly faced with grit substantially exposed to protect said elevated portions. 45
- In testimony whereof I have signed my name in presence of two subscribing witnesses.

MATHIAS B. BECKER.

Witnesses:

M. M. BOYLE,  
G. M. NEVILLE.